

**1**

3,725,195

**PAPERMAKING PROCESS COMPRISING THE INCORPORATION OF A POLYACRYLAMIDE MUCILAGINOUS MATERIAL**

Fujio Suyama and Tokuo Yamamoto, Shizuoka, Kenichi Shimono and Hiroshi Kuwahara, Fuji, Masao Ishii, Tokyo, and Ichiro Watanabe, Yokohama, Japan, assignors to Nitto Chemical Industry Co., Ltd., and Shizuoka-ken, Shizuoka-shi, Japan

No Drawing. Filed Aug. 10, 1970, Ser. No. 62,703

Claims priority, application Japan, Aug. 11, 1969, 44/62,932; Oct. 31, 1969, 44/86,852; Nov. 12, 1969, 44/90,007

Int. Cl. D21h 3/58

U.S. Cl. 162—168

6 Claims

**ABSTRACT OF THE DISCLOSURE**

A process is provided for the preparation of cellulosic paper sheets having a high degree of uniformity. In this process, an improvement has been discovered which comprises (1) sequestering the excess aluminum ion by the addition of a sequestering amount of a member selected from the group consisting of (i) a chelating agent and (ii) an acrylamide-based anionic polymer having a molecular weight of less than 1,000,000; and (2) after sequestering the excess free aluminum ion, then including in said fiber suspension 0.01–2% (based on dry fiber weight) of a polyacrylamide mucilaginous material of a molecular weight of more than 3,000,000 and a hydrolysis degree of 10 to 30%. The process allows the formation of paper sheets of an even texture and quality by obviating the problem of cellulose fiber slippage on the wire mesh and provides a uniform dispersion of the fibers in the vat.

This invention relates to a process for manufacturing paper by use of a synthetic mucilaginous material. Research efforts have been conducted on papermaking by use of a synthetic mucilaginous material for fiber dispersion, anti-freeness and anti-sedimentation, in order to improve uniformity of the paper produced as well as to ensure smooth operation of sheetmaking in manufacturing paper by a paper machine.

For instance, there is found a case where a comparatively low molecular weight water-soluble polyelectrolyte with a strongly anionic property was used. However, when such a polymer is used as a synthetic mucilaginous material, the cellulose fiber is apt to slip down along the surface of cylinder wire, a phenomenon called "wash-off," resulting in poor wet web formation so that a continuous operation of manufacturing paper of sufficient commercial value becomes impossible. Moreover, because of a strong adhesiveness said water-soluble polyelectrolyte tends to adhere to the dryer surface of a paper machine, causing frequent "broke" which renders a continuous operation of papermaking difficult.

On the other hand, although developmental research had been done in the past on making use of polyphosphates, carboxymethylcellulose, sodium alginate and the like as a synthetic mucilaginous material, satisfactory effects of dispersion, anti-freeness and anti-sedimentation on fiber were unattainable and these compounds are currently not in use.

It was only recently that the research on utilization of the polyethylene oxide (hereinafter referred to simply as PEO) as a synthetic mucilaginous material made progress, and this compound is gradually coming into use. However, when said compound was used there arose new difficulties such as a decrease in papermaking speed due to foaming of the stock, necessity of adding an antifoaming agent, a decrease in the sizing effect and in the strength

**2**

of paper, resulting from said addition of an antifoaming agent, and development of unevenness in color which is caused by aggregation of fibers in the paper made from the stock containing dyes. Therefore, development of a novel synthetic mucilaginous material has been desired.

The sheet formation on a cylinder machine takes place as follows: the fiber suspension in a cylinder vat is subjected to suction at the surface of a cylinder wire, and forms wet web on the surface of cylinder as the cylinder rotates. When a synthetic mucilaginous material with insufficient effects of dispersion, anti-freeness and anti-sedimentation on fiber is used, the cellulose fiber tends to slip down along the surface of cylinder wire, a phenomenon called "wash-off"; this results in a poor sheet formation leading to appearance of a strip-pattern in the final paper owing to the differences in thickness between a thick part and a thin part. Further, the synthetic mucilaginous material having excellent effects of dispersion, anti-freeness and anti-sedimentation on fiber is not only necessary for a cylinder machine but also, of course, desirable to be used for a Fourdrinier machine to obtain a satisfactory formation of uniform wet web.

The wash-off can be avoided by suppressing to a certain extent the freeness of the cellulose fiber. As one of the means to judge the degree of suppression of the freeness, there is a method which consists in comparing the difference in liquid levels inside and outside the cylinder. Generally, it is recognized that as said difference becomes greater the wash-off tends to disappear.

The present inventors evaluated various substances as a synthetic mucilaginous material for papermaking by adopting the following procedure as a means to show quantitatively the good or bad sheet formation: The thickness of the final paper was measured at several points situated at regular intervals along the cross-direction of the final paper, and the mean value of these measurements was determined at regular intervals along the machine direction of the paper; from a series of these mean values, the difference in thickness between the thick part and the thin part of the paper was obtained, and this difference served as the basis for the evaluation. As a result, it was found that a polyacrylamide having both of the specific molecular weight and specific hydrolysis degree has a pronounced ability for wet web formation and gives a good result. Based on this finding, the present invention has been accomplished.

The polyacrylamide to be used in this invention should have a hydrolysis degree within the range of 10 to 30%. When a polyacrylamide having a hydrolysis degree of less than 10% is used, the uniformity of the formed sheet tends to become worse; however when the hydrolysis degree exceeds 30% a sticking tendency onto the dryer surface becomes noticeable and dry broke is induced.

Said effect according to the degree of hydrolysis is considered to be due to the influence of the hydrogen bond of the carboxylic group. For example, in the case where the number of carboxylic groups is too small, the number of hydrogen bonds is also small, and it becomes difficult to maintain a uniform state of felting of cellulose fibers produced by the synthetic mucilaginous material, while in the case where the number of carboxylic groups is too large a good result is still obtained as for the sheet formation but a sticking tendency onto the dryer surface becomes stronger and more distinguished than said effect of uniform state of felting, and the sum total of the effects would be only negative.

The molecular weight of polyacrylamide used as a synthetic mucilaginous material in this invention is preferably larger than 3,000,000. When polyacrylamide having a molecular weight less than 3,000,000, for example, a molecular weight of about 2,500,000, is used, the uniformity of formed sheet often becomes inferior, however

controlled the hydrolysis degree of the polymer may be. Although in this case the uniformity of formed sheet may sometimes be improved by the addition of an increased amount of the synthetic mucilaginous material, the addition of a large amount of synthetic mucilaginous material is undesirable from an economical point of view.

Though the amount of the synthetic mucilaginous material used in this invention can be decreased with the increase in the polymerization degree thereof, it is generally effective when present in an amount of 0.01% by weight or more based on the weight of dry fiber. From an economical and other points of view, the preferred amount is 2.0% by weight or less.

The partial hydrolyzate of polyacrylamide used as a synthetic mucilaginous material can be prepared by conventional methods. It may also be prepared by the following procedure:

An aqueous solution containing 3 to 20% by weight of acrylamide monomer is placed in a vessel provided with a reflux condenser; it is allowed to polymerize with stirring under a nitrogen stream using as catalyst 0.01 to 0.1% (based on the weight of monomer) of a persulfate or hydrogen peroxide, or using, if necessary, as a redox catalyst a combination of these compounds with 0.01 to 0.1% by weight of dimethylaminopropionitrile, triethanolamine, sodium thiosulfate, sodium sulfite, ferrous sulfate, or the like. The reaction is run at a temperature of 10° to 50° C. for several to approximately ten hours to obtain an aqueous solution of polyacrylamide. Then, after adding 10 to 30% by mole of a caustic alkali per mole of the polyacrylamide, said solution is stirred at 50° to 90° C. for 2 to 3 hours, to yield a partial hydrolyzate of polyacrylamide having a molecular weight of 3,000,000 or more. The aqueous polymer solution thus obtained has a viscosity of within the range of 100,000 to 500,000 cps. at a concentration of 5%. In actual use, the solution is further diluted to a polymer concentration of 0.001 to 0.1%.

The synthetic mucilaginous material of the present invention cannot be used directly in a rosin-sized stock suspension, because if used, the fibers flocculate so badly that the sheet forming becomes impossible. This phenomenon seems to be caused by the following reasons: the decrease in viscosity due to transformation of the polymer chain of polyacrylamide into a thread-ball-like shape, which is caused by the combination of excess aluminum ion produced by hydrolysis of aluminum sulfate added to fix the rosin sizing agent, with anionic carboxylic groups in the polyacrylamide added as a synthetic mucilaginous material; and the occlusion of fibers in the molecules of the synthetic mucilaginous material when these molecules crimp into a thread-ball-like shape.

The present inventors conducted a research on suppressing the phenomenon of fiber flocculation caused by the aluminum ion existing in excess. As a result, it was found that the phenomenon of fiber flocculation can be suppressed and the present synthetic mucilaginous material can be utilized in forming the sheet from a rosin-sized stock, when said synthetic mucilaginous material is used after the addition of a chelating agent capable of combining ionically with aluminum ion, thereby sequestering the excess free aluminum ion; or after sequestering the excess aluminum ion by the addition of a polymer of the anionic polyacrylamide type having a chain length insufficient to fully occlude fibers when the polymer chain transforms into a thread-ball-like shape.

As said chelating agent for aluminum ion, there are oxalic, malonic, succinic, maleic, malic, tartaric and citric acids, disodium nitrilotriacetate, disodium ethylenediaminetetraacetate, disodium N-oxyethylethylenediaminetetraacetate, disodium 1,2 - diaminocyclohexanetetraacetate, sodium sulfosalicylate and sodium catechol-3,5-disulfonate, etc.

Though the amount of said chelating agent depends upon the amount of excess free aluminum ion, the addi-

tion of 0.05 to 2 moles thereof per mole of aluminum sulfate is generally sufficient.

As a relatively low molecular weight polymer of the acrylamide-type, which also sequesters the excess aluminum ion, there is used an anionic polymer of the polyacrylamide-type having a molecular weight of less than 1,000,000 (hereinafter referred to as "acrylamide-based low molecular polymer"). This polymer is not necessarily limited to a polymer of acrylamide, but a part of acrylamide can be substituted by one or more monomers selected from the group of copolymerizable monomers consisting of (meth)acrylic acid salts, (meth)acrylic acid esters, acrylonitrile, and vinyl acetate. In this case the content of the monomer(s) capable of copolymerizing with acrylamide in the copolymer should be less than 50% by weight. When said content in a copolymer exceeds 50%, there occurs in the course of papermaking an undesirable sticking onto the surface of a dryer of paper machine.

Though the amount of said acrylamide-based low molecular polymer to be used varies according to the amount of aluminum sulfate used in sizing treatment and to its capacity for capturing the aluminum ion, it should be added in an amount of 1 to 10 moles per mole of aluminum sulfate.

The acrylamide-based low molecular polymer used in this invention can be prepared by any known method. It may also be prepared by, for example, the following method: An aqueous solution containing 10 to 25% by weight of the monomer is placed in a vessel provided with a reflux condenser, and allowed to polymerize with stirring while nitrogen is being blown in, using as catalyst 0.05 to 10% by weight (based on the weight of monomer) of a persulfate or hydrogen peroxide, or using, if necessary, as redox catalyst a combination of these compounds with 0.05 to 10% by weight of dimethylaminopropionitrile, triethanolamine, sodium thiosulfate, sodium sulfite, ferrous sulfate, or the like, at a temperature of 20° to 70° C. for one to several hours to complete the polymerization and to obtain an aqueous solution of the polymer. Those polymers which contain no carboxylic group in the molecule are further heated with stirring after addition of a caustic alkali in an amount corresponding to 1 to 30% by mole, at 50° to 90° C. for 1 to 3 hours to obtain a partial hydrolyzate of the polymer. The aqueous polymer solution thus obtained has a viscosity of within the range of 100 to 20,000 centipoise (cps.), as measured by a Brookfield viscometer at a polymer concentration of 10%. In actual use, said solution is further diluted to a polymer concentration of 0.5 to 5%.

The above-mentioned chelating agent or acrylamide-based low molecular polymer, which serves to sequester the excess free aluminum ion in rosin-sized stock is added to the stock subsequent to the sizing treatment with a rosin sizing agent and aluminum sulfate, and then a polyacrylamide having a molecular weight of more than 3,000,000 and a hydrolysis degree of 10 to 30% is added thereto, whereupon the sheet formation can be started, thus leading to an extremely smooth operation of making even a rosin-sized paper.

By use of the present synthetic mucilaginous material, the uniformity of final paper is improved, the sheet-forming proceeds smoothly, and because of lack of flocculation of fibers the unevenness in color, which is attributable to the flocculation of dyed fibers, is entirely prevented, whereas said unevenness in color is observed in the case where polyethylene oxide is used in a dyed stock.

The present invention is further illustrated hereunder with reference to examples. In the examples, the measurement of dispersion level was evaluated from the light transmittance at 660 m $\mu$  by use of a photoelectric colorimeter. The testing of sizing degree was conducted according to the method of JIS P 8122. The testing of water

absorption degree was conducted in accordance with the method specified in JIS P 8141.

## EXAMPLE 1

In a Hollander beater 40 kg. of a commercial NBKP (coniferous bleached kraft pulp) was beated at a consistency of 3% (by weight; the same shall apply hereinafter) for one hour to a Canadian freeness of 650 to 700 cc. Then the stock was diluted to a consistency of 0.1%, and sent to a cylinder vat where the diluted stock was admixed with an aqueous polyacrylamide solution which had previously been diluted to a concentration of 0.1%. From the stock was made a tissue paper of 16.0 g./m.<sup>2</sup> basis weight. The results of tests conducted on the final paper thus prepared were summarized in Table 1. The paper machine used was a cylinder Yankee machine of the uniflow type, and the width of sheet-forming was 445 mm.

Among the results of tests shown in Table 1, the rating of sheet formation was obtained as follows: by means of a micrometer a set of thickness measurements was made at 5 points spaced at every 5 cm. interval in a line along the cross direction of the sheet, commencing at a point 12.25 to the left edge of the sheet; a number of these sets of measurements were done along the machine direction of the sheet at every 2.5 cm. interval; the mean values of thicknesses of each set were determined and the difference between the maximum and the minimum mean values was taken as the criterion in the following manner: "excellent" for the difference of 1 $\mu$  or less, "good" for 1.1 to 1.5 $\mu$ , "fair" for 1.6 to 2.0 $\mu$ , and "poor" for 2.1 $\mu$  or more. In the sheet marked "poor" in this evaluation method, there was observed by visual inspection also a stripe pattern so distinct that the sheet was of no commercial value.

In a Niagara beater, 650 g. of a commercial NBKP was beated at a consistency of 3% for 30 minutes to a Canadian freeness of 690 cc. After completion of the beater treatment, the stock was admixed with 1.0% (100% basis; the same shall apply hereinafter) on the basis of dry fiber of a rosin sizing agent and 0.9% on the basis of dry fiber of aluminum sulfate (containing 18 molecules of water of crystallization; the same shall apply hereinafter), and thoroughly mixed with stirring. The pH of the stock thus treated was 4.5.

Subsequently, as given in Table 3, disodium nitrilotriacetate (NTA-2Na) was added to the stock as a chelating agent in an amount of 1 to 2 moles per mole of added aluminum sulfate, and the stock was diluted to a consistency of 0.1%. A definite quantity of said diluted stock was admixed with 2% on the basis of dry fiber of a high-molecular weight polyacrylamide having a molecular weight of 5,000,000 and a hydrolysis degree of 20%, which had been prepared in advance. The measurement of dispersion level of fibers was evaluated from the light transmittance at 660 m $\mu$  by use of a photoelectric colorimeter. On the other hand, the results of visual inspection were shown along with the light transmittance in the table, where "poor" means distinct appearance of flocculation and "good" means no flocculation on adding the synthetic mucilaginous material.

35

TABLE 1

| Run No. | Polyacrylamide          |                             | Freeness of the stock in vat admixed with synthetic mucilaginous material (cc.) | Head difference between inside and outside of cylinder (mm.) | Machine speed (m./min.) | Frequency of adherence to dryer | Rating of sheet formation (U) | Basis weight (g./m. <sup>2</sup> ) |
|---------|-------------------------|-----------------------------|---------------------------------------------------------------------------------|--------------------------------------------------------------|-------------------------|---------------------------------|-------------------------------|------------------------------------|
|         | Mol. wt. 1,000 $\times$ | Degree hydrolysis (percent) |                                                                                 |                                                              |                         |                                 |                               |                                    |
| 1-----  | 5,000                   | 5                           | 1.40                                                                            | 510                                                          | 8                       | 41.3                            | Small.....                    | Poor (2.1)-----                    |
| 2-----  | 5,000                   | 10                          | 1.01                                                                            | 480                                                          | 14                      | 40.9                            | do.....                       | Good (1.25)-----                   |
| 3-----  | 5,000                   | 20                          | 0.65                                                                            | 510                                                          | 20                      | 43.6                            | do.....                       | Excellent (0.75)-----              |
| 4-----  | 5,000                   | 30                          | 0.67                                                                            | 490                                                          | 20                      | 41.0                            | Medium.....                   | Excellent (0.80)-----              |
| 5-----  | 5,000                   | 40                          | 0.65                                                                            | 490                                                          | 20                      | 40.8                            | Large.....                    | Excellent (0.79)-----              |
| 6-----  | 3,000                   | 20                          | 1.88                                                                            | 525                                                          | 15                      | 40.0                            | Small.....                    | Fair (1.95)-----                   |
| 7-----  | 2,600                   | 20                          | 2.50                                                                            | 520                                                          | 12                      | 40.0                            | do.....                       | Poor (2.30)-----                   |

## EXAMPLE 2

A commercial NUKP (coniferous unbleached kraft pulp) was charged in a TAPPI-Standard Niagara beater, and beated at a consistency of 3% for 3 hours to a Canadian freeness of 300 cc. Then, each of the dyestuffs listed in Table 2 was separately added to the stock in an amount of 1.0 to 5.0% on the basis of dry fiber, and thoroughly mixed with stirring. After being added with a polyacrylamide (molecular weight, 5,000,000; degree of hydrolysis, 20%), which had been diluted to a concentration of 0.1%, or with a polyethylene oxide, which also had been diluted to a concentration of 0.1%, each in an amount of 0.01% on the basis of dry fiber, each stock were made into handmade sheets by means of a square-type sheet machine. The final sheets were compared for the flocculation of colored fibers, and the results obtained were as shown in Table 2.

TABLE 2

| Run No. | Name of dyestuff     | Amount of dye added, percent | Presence of flocculation of colored fibers |                |
|---------|----------------------|------------------------------|--------------------------------------------|----------------|
|         |                      |                              | Polyethylene oxide                         | Polyacrylamide |
| 1-----  | Diacotton Congo Red  | 1.5                          | Yes.....                                   | No.....        |
| 2-----  | Direct Deep Black GX | 5.0                          | Yes.....                                   | No.....        |
| 3-----  | Direct Dark Green B  | 1.5                          | Yes.....                                   | No.....        |
| 4-----  | Direct Green B       | 1.5                          | Yes.....                                   | No.....        |
| 5-----  | Direct Bron 3G       | 1.0                          | Yes.....                                   | No.....        |

## EXAMPLE 3

In a Niagara beater, 650 g. of a commercial NBKP was beated at a consistency of 3% for 30 minutes to a Canadian freeness of 690 cc. After completion of the beater treatment, the stock was admixed with 1.0% (100% basis; the same shall apply hereinafter) on the basis of dry fiber of a rosin sizing agent and 0.9% on the basis of dry fiber of aluminum sulfate (containing 18 molecules of water of crystallization; the same shall apply hereinafter), and thoroughly mixed with stirring. The pH of the stock thus treated was 4.5.

Subsequently, as given in Table 3, disodium nitrilotriacetate (NTA-2Na) was added to the stock as a chelating agent in an amount of 1 to 2 moles per mole of added aluminum sulfate, and the stock was diluted to a consistency of 0.1%. A definite quantity of said diluted stock was admixed with 2% on the basis of dry fiber of a high-molecular weight polyacrylamide having a molecular weight of 5,000,000 and a hydrolysis degree of 20%, which had been prepared in advance. The measurement of dispersion level of fibers was evaluated from the light transmittance at 660 m $\mu$  by use of a photoelectric colorimeter. On the other hand, the results of visual inspection were shown along with the light transmittance in the table, where "poor" means distinct appearance of flocculation and "good" means no flocculation on adding the synthetic mucilaginous material.

35

TABLE 3

| Item                                                               | Run number                                                                                                               |      |      |  |
|--------------------------------------------------------------------|--------------------------------------------------------------------------------------------------------------------------|------|------|--|
|                                                                    | 1                                                                                                                        | 2    | 3    |  |
| Conditions in common                                               | NBKP=100 %<br>Canadian freeness=690 cc.<br>Amount of rosin sizing agent added=1.0%<br>Aluminum sulfate=0.97%<br>(pH=4.5) |      |      |  |
| Amount of NTA-2Na added (moles per mole of aluminum sulfate added) | 0                                                                                                                        | 1.0  | 2.0  |  |
| Dispersion level;                                                  |                                                                                                                          |      |      |  |
| Light transmittance (percent)                                      | 93.5                                                                                                                     | 42.0 | 41.5 |  |
| Visual inspection                                                  | Poor                                                                                                                     | Good | Good |  |
| Stockigt sizing degree (sec.)                                      | 7.7                                                                                                                      | 7.7  | 7.8  |  |

## EXAMPLE 4

To the stock treated in a beater in the manner similar to that in Example 3, 1.0% on the basis of dry fiber of a rosin sizing agent and 0.9% on the basis of dry fiber of aluminum sulfate were added to fix the rosin sizing agent at pH 4.5, and then the stock was diluted to a consistency of 0.1%. Each definite quantity of said diluted stock was added with, as a sequestering agent for aluminum ion, 1 to 2 moles of sodium sulfosalicylate (SSA-Na) per mole of aluminum sulfate used for fixing the rosin sizing agent. The dispersion degree of fibers was evaluated by

measuring the light transmittance with a photoelectric colorimeter. On the other hand, the results of visual inspection were also given in the table, wherein "poor" means distinct occurrence of flocculation on adding the

"good" means absence of such phenomenon of flocculation. In order to test the sizing degree a test sheet is prepared, and in this example it was prepared by hand-making.

TABLE 5

| Item                                                                                                                   | Run number |      |                  |      |      |      |
|------------------------------------------------------------------------------------------------------------------------|------------|------|------------------|------|------|------|
|                                                                                                                        | 1          | 2    | 3                | 4    | 5    | 6    |
| (NBKP=100%<br>Canadian freeness=690 cc.<br>Amount of rosin sizing agent added=1.0%<br>Aluminum sulfate=0.9%<br>pH=4.5) |            |      |                  |      |      |      |
| Amount of low molecular weight polyacrylamide added (moles per mole of aluminum sulfate added)-----                    | 0          | 0    | 2                | 3    | 5    | 10   |
| Dispersion level:                                                                                                      |            |      |                  |      |      |      |
| Light transmittance (percent)-----                                                                                     | 62.5       | 73.5 | 52.2             | 41.1 | 40.5 | 40.5 |
| Visual inspection-----                                                                                                 | Poor       | Poor | ( <sup>1</sup> ) | Good | Good | Good |
| Stöckigt sizing degree (sec.)-----                                                                                     | 7.7        | 7.7  | 15.0             | 15.9 | 18.5 | 18.8 |

<sup>1</sup> Fairly good.

NOTE.—Run No. 1 in the table is the case where both low molecular weight polyacrylamide and synthetic mucilaginous material are absent. Run No. 2 in the table is the case wherein a synthetic mucilaginous material alone was added without adding a low molecular weight polyacrylamide.

synthetic mucilaginous material, and "good" means no such flocculation.

TABLE 4

| Item                                                                                                   | Run number |      |      |
|--------------------------------------------------------------------------------------------------------|------------|------|------|
|                                                                                                        | 1          | 2    | 3    |
| (NBKP=100%<br>pH=4.5<br>Canadian freeness 690 cc.<br>Rosin sizing agent=1.0%<br>Aluminum sulfate=0.9%) |            |      |      |
| Amount of SSA-Na added (moles per mole of aluminum sulfate added)-----                                 | 0          | 1.0  | 2.0  |
| Dispersion level:                                                                                      |            |      |      |
| Light transmittance (percent)-----                                                                     | 93.0       | 41.5 | 41.0 |
| Visual inspection-----                                                                                 | Poor       | Good | Good |
| Stöckigt sizing degree (sec.)-----                                                                     | 7.7        | 7.8  | 7.8  |

The Stöckigt sizing degree in Tables 3 and 4 was determined on a specimen of paper made on a TAPPI Standard sheet machine.

The same stock as that in Example 3 was added with 1.0% of a rosin sizing agent and 0.9% of aluminum sulfate, and thoroughly mixed with stirring to fix the rosin sizing agent while maintaining pH at 4.5. Then a low molecular weight polyacrylamide having a molecular weight of 700,000 was added in an amount of 2 to 10 moles per mole of aluminum sulfate added for fixing, and diluted to a consistency of 0.1%. Each portion of definite quantity of the diluted stock was admixed with 1% on the basis of dry fiber of a high molecular weight polyacrylamide having a molecular weight of 9,000,000 and a hydrolysis degree of 20%, and made into sheet in the manner similar to that in Example 5 in order to evaluate the dispersion level of fibers. The test was conducted in the manner similar to that in Example 5, and the results were as shown in Table 6.

TABLE 6

| Item                                                                                                                   | Run number |      |      |      |      |      |
|------------------------------------------------------------------------------------------------------------------------|------------|------|------|------|------|------|
|                                                                                                                        | 1          | 2    | 3    | 4    | 5    | 6    |
| (NBKP=100%<br>Canadian freeness=690 cc.<br>Amount of rosin sizing agent added=1.0%<br>Aluminum sulfate=0.9%<br>pH=4.5) |            |      |      |      |      |      |
| Amount of low molecular weight polyacrylamide added (moles per mole of aluminum sulfate added)-----                    | 0          | 0    | 2    | 3    | 5    | 10   |
| Dispersion level:                                                                                                      |            |      |      |      |      |      |
| Light transmittance (percent)-----                                                                                     | 62.6       | 73.5 | 45.4 | 40.0 | 39.5 | 40.0 |
| Visual inspection-----                                                                                                 | Poor       | Poor | Good | Good | Good | Good |
| Stöckigt sizing degree (sec.)-----                                                                                     | 7.7        | 7.7  | 13.5 | 18.8 | 23.3 | 25.5 |

NOTE.—Run No. 1 in the table is the case where both low molecular weight polyacrylamide and synthetic mucilaginous material are absent. Run No. 2 in the table is the case wherein a synthetic mucilaginous material alone was added without adding a low molecular weight polyacrylamide.

EXAMPLE 5

To the stock treated in a beater in the manner similar to that in Example 3, 1.0% on the basis of dry fiber of a commercial rosin sizing agent and 0.9% on the basis of dry fiber of aluminum sulfate were added, and thoroughly mixed with stirring while maintaining pH at 4.5 to fix the rosin sizing agent.

Subsequently, as shown in Table 5, a low molecular weight polyacrylamide having a molecular weight of 200,000 was added to each portion of the stock in an amount of 2 to 10 moles per mole of aluminum sulfate added to fix the rosin sizing agent, and each portion of the stock was diluted to 0.1% consistency. To the stock was added 2% on the basis of dry fiber of a synthetic mucilaginous material having a molecular weight of 5,000,000 and a hydrolysis degree of 20%. After elapse of a definite time, the turbidity of the stock suspension was measured with a photoelectric colorimeter in knowing the dispersion level of fibers. On the other hand, the results of visual inspection were also given in the table, wherein "poor" means distinct occurrence of flocculation of fibers on adding a polyacrylamide having a molecular weight of 5,000,000 and a hydrolysis degree of 20%, and

55 In a Hollander beater 40 kg. of a commercial NBKP was beaten at a consistency of 3% for one hour to a Canadian freeness of 670 cc. to obtain a stock.

60 To the stock were added 1% on the basis of dry fiber of a commercial rosin sizing agent and 1.0 to 2.6% on the basis of dry fiber of aluminum sulfate were added, and thoroughly mixed to fix the rosin. The pH of the stock was 4.4 to 4.8. Each rosin sized stock was diluted to 0.1% consistency, and sent to the vat of a cylinder machine, where a low molecular weight polymer of the acrylamide type composed of 95% of acrylamide and 5% of sodium acrylate and having a molecular weight of 200,000, or the one composed of 80% of acrylamide, 10% of acrylonitrile and 10% of sodium acrylate and having a molecular weight of 700,000 was added thereto in order to sequester the aluminum ion. Then, to each stock was added as a synthetic mucilaginous material an aqueous solution of a high molecular weight polyacrylamide having a molecular weight of 5,000,000 and a hydrolysis degree of 20% (abbreviated as PAA-a), or 65 of a high molecular weight polyacrylamide having a

EXAMPLE 7

molecular weight of 9,000,000 and a hydrolysis degree of 20% (abbreviated as PAA-b), both solutions having been previously prepared by dilution to a concentration of 0.1%. From each stock tissue papers were prepared.

One each final paper thus prepared, the test for water absorption degree (period of immersion, 10 min.) was made to obtain the results as shown in Table 7. The machine used was a cylinder Yankee machine of the uniflow type, and the width of sheet-forming was 445 mm.

3. A process according to claim 2, wherein said chelating agent is disodium ethylenediaminetetraacetate, disodium nitrilotriacetate, citric acid, tartaric acid or sodium sulfosalicylate.

5 4. A process according to claim 1, wherein said wet web is admixed with said acrylamide-based anionic polymer which is polyacrylamide in an amount of 1 to 10 moles per mole of aluminum sulfate.

10 5. A process according to claim 1, wherein said wet web is admixed with an acrylamide-based anionic poly-

TABLE 7

| Item                                                                          | Run number |      |       |         |      |       |      |
|-------------------------------------------------------------------------------|------------|------|-------|---------|------|-------|------|
|                                                                               | 1          | 2    | 3     | 4       | 5    | 6     | 7    |
| Amount of sizing agent added (percent).....                                   | 1.0        | 1.0  | 1.0   | 1.0     | 1.0  | 1.0   | 1.0  |
| Aluminum sulfate added (percent).....                                         | 2.6        | 1.0  | 1.0   | 1.0     | 1.0  | 1.0   | 1.0  |
| DH in the stock.....                                                          | 4.4        | 4.6  | 4.6   | 4.6     | 4.6  | 4.6   | 4.6  |
| Polymerization degree of low molecular weight polymer of acrylamide type..... | 200,000    |      |       | 700,000 |      |       |      |
| Amount of the above polymer added (moles per mole of aluminum sulfate).....   | 0          | 2.0  | 3.0   | 5.0     | 2.0  | 3.0   | 5.0  |
| Kind of synthetic mucilaginous material.....                                  | PEO        |      | PAA-a |         |      | PAA-b |      |
| Amount of the above agent added (percent).....                                | 0.62       |      | 1.4   |         |      | 0.7   |      |
| Head difference between inside and outside of the cylinder (mm).....          | 22         | 25   | 25    | 25      | 24   | 24    | 24   |
| Basis weight (g./m. <sup>2</sup> ).....                                       | 18.2       | 12.2 | 12.8  | 12.3    | 12.3 | 12.5  | 12.8 |
| Water absorption degree (mm).....                                             | 6          | 2    | 2     | 2       | 3    | 2     | 2    |

What is claimed is:

1. In a process for the preparation of cellulosic paper sheets having a high degree of uniformity through the steps of

- (a) forming a cellulosic fiber suspension in a vat, said cellulosic fiber stock having been sized with a rosin sizing agent and aluminum sulfate;
- (b) subjecting said suspension to suction at the surface of said vat through a wire mesh, whereby a wet web of said cellulosic fiber is formed; and
- (c) preparing a finished sheet of paper from said wet web

the improvement which comprises (1) sequestering the excess aluminum ion by the addition of a sequestering amount of a member selected from the group consisting of (i) a chelating agent and (ii) an acrylamide-based anionic polymer having a molecular weight of less than 1,000,000; and (2) after sequestering the excess free aluminum ion, the inclusion in said fiber suspension of an effective amount of a synthetic mucilaginous material to provide for the formation of paper sheets of an even texture and quality by obviating the problem of cellulose fiber slippage on said wire mesh and providing a uniform dispersion of the fibers in the vat, said synthetic mucilaginous material being a polyacrylamide of a molecular weight of more than 3,000,000 and a hydrolysis degree of 10 to 30%, and said effective amount being from 0.01 to 2% based on the weight of the dry fiber.

2. A process according to claim 1, wherein said wet web is admixed with said chelating agent in an amount of 0.05 to 2 moles per mole of aluminum sulfate.

30 mer which is a copolymer composed of acrylamide and less than 50% by weight based on total weight of monomers of at least one member selected from the group consisting of acrylic acid salts, methacrylic acid salts, acrylic acid esters, methacrylic acid esters, acrylonitrile, and vinyl acetate, in an amount of 1 to 10 moles per mole of aluminum sulfate.

35 6. A process according to claim 5 wherein the acrylic and methacrylic acid salts are members selected from the group consisting of the sodium, potassium and ammonium salts and the acrylic and methacrylic acid esters are members selected from the group consisting of the methyl, ethyl, n-propyl and n-butyl esters.

#### References Cited

#### UNITED STATES PATENTS

|              |         |                      |           |
|--------------|---------|----------------------|-----------|
| 3,076,740    | 2/1963  | Reynolds et al. .... | 162—168 X |
| 3,019,157    | 11/1962 | Reynolds et al. .... | 162—180 X |
| 3,391,057    | 7/1968  | Spence et al. ....   | 162—168 X |
| 50 3,433,659 | 3/1969  | D'Errico et al. .... | 162—180 X |
| 3,112,242    | 11/1963 | Jones ....           | 162—180 X |
| 3,332,834    | 7/1967  | Reynolds ....        | 162—168 X |
| 3,255,072    | 6/1966  | Sheetz ....          | 162—168   |

ROBERT L. LINDSAY, JR., Primary Examiner

F. FREI, Assistant Examiner

U.S. Cl. X.R.

162—158, 180, 183